

## UNITED STATES PATENT OFFICE

RUPERT S. DANIELS, OF NEWARK, NEW JERSEY, ASSIGNOR TO BAKELITE CORPORATION, OF NEW YORK, N. Y., A CORPORATION OF DELAWARE

## WATER REPELLENT ABRASIVE

No Drawing.

Application filed September 15, 1928. Serial No. 306,292.

This invention relates to abrasives for use in wet grinding and more particularly to porous abrasive or grinding wheels for use with water under conditions where the temperature of the water is apt to reach 100° C.

Artificial abrasive wheels and other like implements are prepared from abrasive grit and a binder. A binding medium in extensive use for this purpose is the synthetic resinous material obtained, for example, in the condensation of a phenol with formaldehyde or its equivalent or other aldehydes, which is designated as a resinoid on account of its characteristic difference from the true resins in that it polymerizes upon heating to a form that is infusible and insoluble for all practical purposes. Such abrasive wheels are made more or less porous in order that they may be effective for free cutting and lose about 75 per cent of their strength when run in hot or boiling water which is necessary for certain industrial purposes; as a consequence they are practically useless under such conditions.

I have discovered that this loss in strength in the presence of hot or boiling water can be materially reduced or avoided without affecting the free cutting action of a porous grinding wheel by the impregnation of the wheel with a substance which has a melting point above 100° C. and which is water repellent. In other words, I have found it to be essential in preventing material loss in strength of the wheel that the impregnating material should not be caused to flow from the wheel or be leached out or otherwise affected by hot or boiling water.

Very suitable impregnating materials which satisfy these conditions are the wax-like higher chlorinated naphthalenes or mixtures thereof, which are substantially free from mono- and dichlor-naphthalenes and have melting points above 100° C. It is not enough, however, that the melting point be high, for a pitch which remains after distillation of chlorinated naphthalene up to 355° C. still contains enough material that is soluble in boiling water so as to render it ineffective as a water repellent; on this ac-

count the impregnating material must also be substantially insoluble in boiling water.

A mixture of tri-chlor- and tetra-chlor-naphthalenes having a melting point of approximately 107° C. (found by melting and then allowing to cool to constant temperature) is generally suitable, provided it is substantially free from dichlor-naphthalene and other objectionable admixtures though boiling water seems to have a slight softening action on the wax-like mass. A preferable mixture is one consisting largely of pentachlor-naphthalene which solidifies at about 126° C. and which is not affected by boiling water. The removal of the dichlor-naphthalene, which is present in the various chlorinated naphthalene wax mixtures in objectionable amounts, is necessary as otherwise the mixture tends to soften and is not effective as a water repellent when in contact with boiling water.

A procedure which is suitable for the impregnation of abrasive wheels comprises preparing a bath of the impregnating wax at a temperature about 15 degrees above its melting point in a closed chamber, heating a wheel to about 135° C., immersing it in the molten wax, and applying a partial vacuum corresponding to about 28 inches of mercury. The wheel is left in the wax until bubbling ceases and then the temperature of the wax is lowered almost to its solidification point. As the wheel is removed from the bath, it is passed in front of a cooling air current whereupon the wax immediately hardens so that there is no loss from drippage. Excess wax on the surface is then removed. Wheels so impregnated have been found to increase from 12 to 17 per cent in weight. Other methods of impregnation known to the art may be substituted, it being desirable that the voids existing in the porous wheel be filled as completely as possible with the wax.

Wheels, which before impregnation lose about 75 per cent of their strength when run in boiling water, show only a 10 per cent or less loss after impregnation with the above mentioned waxes. Furthermore, the substances herein designated as suitable for impregnation are not affected by dilute alka-

lies, although the resinoid binder may be. Therefore, the impregnating materials perform the additional function of protecting the resinoid binder when alkaline solutions 5 are used in grinding operations. In addition the above mentioned chlornaphthalene compounds act as lubricants at the cutting points, thus increasing the efficiency of the wheel, and prevent filling of the pores with ground 10 material. The temperature of the wheel when it is run in boiling water does not reach that of the melting point of the impregnating material and consequently there is no flow of the impregnating material from the wheel.

15 While the above disclosure is more specifically directed to grinding wheels, the invention is also applicable to the manufacture of abrasive paper and other abrasive implements. Moreover, it is evident that this in- 20 vention is not limited to abrasives bonded by means of phenol resinoids, but that other suitable types of binders known in the art, such as for example the glycerol-phthalic an- 25 hydride resinoids, suitable silicates, car- bamid or thiocarbamid resinoids, cellulose esters, etc., may be used so long as they can be manipulated to yield an implement which can be impregnated.

I claim:

30 1. An abrasive implement for wet grinding having a porous structure prepared from abrasive particles bonded with a resinoid and impregnated with chlorinated naphthalene which is substantially free from mono- and 35 dichlornaphthalenes.

2. An abrasive implement for wet grinding having a porous structure prepared from abrasive particles bonded with a phenol- 40 formaldehyde resinoid and impregnated with chlorinated naphthalene comprising largely pentachlornaphthalene and substantially free from mono- and dichlornaphthalenes.

In testimony whereof, I affix my signature

RUPERT S. DANIELS

45

50

55